

## [54] CIGARETTE AND FILTER

[75] Inventor: Harold Grossman, Silver Spring, Md.

[73] Assignee: Montclair Research Corporation,  
Silver Spring, Md.

[21] Appl. No.: 862,212

[22] Filed: Dec. 19, 1977

## Related U.S. Application Data

[60] Continuation-in-part of Ser. No. 687,109, May 17,  
1976, abandoned, which is a division of Ser. No.  
479,104, Jun. 13, 1974, abandoned.[51] Int. Cl.<sup>2</sup> ..... A24B 15/00[52] U.S. Cl. ..... 131/261 R; 131/10 R;  
55/103; 55/523; 55/527[58] Field of Search ..... 131/266, 267, 261, 8,  
131/9, 10, 268, 17 R, 269; 55/103, 523, 527

## [56] References Cited

## U.S. PATENT DOCUMENTS

3,087,500 4/1963 Jacobson ..... 131/17 R

3,127,901 4/1964 Whitfield et al. ..... 131/267  
3,251,365 5/1966 Keith et al. ..... 131/10.9

## FOREIGN PATENT DOCUMENTS

654994 7/1951 United Kingdom ..... 131/10.9  
752358 2/1954 United Kingdom ..... 131/266  
1070437 6/1967 United Kingdom ..... 131/17 R

Primary Examiner—Robert W. Michell

Assistant Examiner—V. Millin

Attorney, Agent, or Firm—Shapiro and Shapiro

## [57] ABSTRACT

A filter for tobacco smoke employs synthetic, inorganic, water-insoluble, anhydrous fibers having a positive zeta potential at the pH of tobacco smoke.

To increase the effectiveness of the filter, the tobacco associated with the filter has mixed therewith and deposited thereon particles of a water-insoluble, hydrophobic, moisture-laden, negative charge-imparting substance.

11 Claims, 1 Drawing Figure



FIG. 1



## CIGARETTE AND FILTER

This application is a continuation-in-part of Application Ser. No. 687,109 filed May 17, 1976 now abandoned, which is a divisional of Application Ser. No. 479,104 filed June 13, 1974, now abandoned.

The invention relates to improvements in filters for tobacco smoke, and to the combination of a body of divided tobacco which is treated to make the filter associated with the tobacco more effective.

### BACKGROUND OF THE INVENTION

Cigarette filters now in commercial use are only partially effective; they remove approximately 30% of the tars and nicotine. The approximately 70% that passes the filter obviously is not trapped by the filter material. The reason is that these substances are in the form of fine particles which are colloidally dispersed, and because of their small size pass through the usual or known filters with the gases in which they are dispersed.

Tobacco smoke is a two-phase system: a vapor phase and a dispersed particulate phase. The vapor phase may be considered the fraction which is volatile above 86° F., which is smoking temperature, and some high boiling point components not immediately condensed. The smoke consists of approximately 4-9% particulate matter or particles dispersed in the 91-96% vapor phase components. The vapor phase components consist of nitrogen, oxygen, carbon monoxide gases and other materials which are in the gaseous state above 86° F. During the smoking process, pyrolysis, pyrolysis, and distillation take place, and it has been estimated that there are as many as 700-800 resulting compounds. Straight chain hydrocarbons predominate.

When a cigarette is being smoked, the particulates which are generated have Brownian movement within the gaseous vapor phase. Observations with a dark field condenser, dialysis, electrophoresis, and Tyndal studies indicate that many particulates in the smoke are negatively charged and have lively Brownian motion. It has been estimated that there are approximately  $2 \times 10^9$  negatively charged particles per millimeter in tobacco smoke.

Also, one of the serious problems in the filtration of tobacco smoke is the hydrophobic character of the carcinogenic tars, which are oleophilic.

### SUMMARY OF THE INVENTION

In accordance with the invention, a filter for tobacco smoke is provided which acts to attract the negatively charged particles dispersed in tobacco smoke. The filter is made of synthetic, inorganic, water-insoluble, anhydrous fibers which have a positive zeta potential at the pH of tobacco. The fibers may be hydrophobic or hydrophilic.

Based upon tests and observations, filters made in accordance with the invention act to cause coalescence of the colloidally dispersed negative particles in the smoke to enlarge them and render them more easily filterable. By coalescing the particles to shift the size distribution to the larger portion of the size-distribution curve, much more effective filtration is accomplished. As the size of the coalesced particles increases, the mass becomes larger thereby decreasing the number of particles in the smoke. Increasing the mass, increases the probability of the particles contacting the absorber sur-

face of the filter. As the diameter of the coalesced mass of particles increases, the distance from the particle to the absorbing surface provided by the individual fibers becomes shorter. The universal gravitational attraction increases; also, the electrostatic forces between the larger coalesced particles and the fibers are increased. Since removal of particulates in smoke depends on probability of collision or contact with the fiber absorber surfaces, the probabilities are increased with increased particle size. This is essentially a physical phenomenon. The velocity of flow of the larger particles is slower than that of the smaller particles. Increased mass decreases the velocity of the particles in the gas flow. The larger the mass, the greater the initial impaction which is a major influence in filter efficiency. Thus, by causing the colloidally dispersed negative particles in the smoke to be coalesced into clumps of increased size and mass, marked improvement in filter efficiency is attained.

To increase the efficiency of the filter, the positive charge or the positive zeta potential on the fibers may be increased by coating the fibers with a secondary source of positive zeta potential. This boosting or enhancement of the positive zeta potential is accomplished by adding to the fibers a positive colloidal metal oxide or a metal oxide having more than one positive ion.

In order to substantially increase the effectiveness of the filter, the tobacco with which the filter is associated is treated so that in the burning the resulting smoke will contain more particulates which are negatively charged, also more strongly negatively charged, in addition to the particulates which normally are negatively charged. For this purpose, the tobacco has deposited thereon particles of a water-insoluble, hydrophobic, moisture-laden, negative charge-imparting substance.

These, and other objects and advantages of the invention will be apparent from the following detailed description, taken in conjunction with the drawing.

### BRIEF DESCRIPTION OF THE DRAWING

FIG. 1 is a graph showing the zeta potential of fibers suitable for making the filter of the invention.

### DESCRIPTION OF THE PREFERRED EMBODIMENT

To increase the size of the particles suspended in the smoke or vapor phase, or to cause their coalescence, a filter made in accordance with the invention comprises synthetic, inorganic, water-insoluble, anhydrous fibers having a positive zeta potential at the pH of tobacco smoke. The positive charge on the fibers attracts the negative charge on the suspended particles, neutralizing them and causing coalescence into clumps of larger size and reducing the number of particle units.

In greater detail, the filter which has furnished outstanding results is made of alumina fibers and which, of course, has the aforementioned properties and characteristics. Such fibers are marketed by ICI America, Inc., Wilmington, Delaware 19899, under the trademark "Saffil". As indicated in FIG. 1, in the pH zone for tobacco smoke, which is approximately 3-6, alumina fibers have a positive zeta potential of between approximately 48-50 millivolts, a strong positive charge. The other significant property of this fiber is that it has a large surface area for absorption, 100-150m<sup>2</sup>/g, as measured by BET/nitrogen absorption. The mean fiber diameter is 3μ, with about 95% of the fibers within the

range of  $1-5\mu$ . Other significant properties are fiber density  $2.8\text{g}/\text{cm}^3$ ; melting point in excess of  $2,000^\circ\text{C}$ ; and tensile strength  $150 \times 10^3\text{psi}$ .

Although the results were not as superior as furnished with filters made with the high absorption alumina, good results were obtained with a filter made of zirconia fibers. Such fibers are also marketed by ICI America, Inc., under the same "Saffil" trademark. Referring to FIG. 1, zirconia has a positive zeta potential between approximately 50-65. The absorption of zirconia, however, is less than the absorption of alumina, being  $5-15\text{m}^2/\text{g}$ . Fibers are made of the same diameter as alumina fibers. The fiber density for zirconia fibers is  $5.6\text{g}/\text{cm}^3$ ; the melting point is in excess of  $2,500^\circ\text{C}$ . and the tensile strength is  $100 \times 10^3\text{psi}$ .

Another synthetic, inorganic, water-insoluble, anhydrous fiber resistant to temperatures of at least approximately  $800^\circ\text{C}$ . is an alumina-silica fiber made by Babcock & Wilcox, and sold under the trademark "Kao-wool". This fiber is available in an average diameter of 2.8 microns and at an average length of 4 inches. It will withstand a temperature of  $2,300^\circ\text{F}$ . and has a tensile strength of  $1.9 \times 10^5\text{psi}$ . The fiber has a specific gravity of 2.56. This fiber consists of approximately 45%  $\text{Al}_2\text{O}_3$ , 52%  $\text{SiO}_2$ , 1.3%  $\text{Fe}_2\text{O}_3$ , 1.7%  $\text{TiO}_2$  and traces of  $\text{MgO}$ ,  $\text{CaO}$ ,  $\text{Na}_2\text{O}$ , and  $\text{B}_2\text{O}_3$ . The positive zeta potential for this fiber is low as compared to the positive zeta potential for the alumina and zirconia fibers; that is, it is only approximately +8 to -6 millivolts in the pH zone for tobacco smoke. This fiber, however, has the advantage of being available in comparatively long lengths, and its positive zeta potential may be enhanced by a positive zeta potential enhancing agent as subsequently described. Also, this fiber is highly suitable for mixture with the high positive zeta potential alumina or zirconia fibers.

The described fibers are made into rod-like form of suitable diameter and density and enveloped in suitable material as known in the art to furnish cigarette filters when cut to predetermined lengths. From the indicated densities, the fibers are very fluffy, and a suitable filter for a cigarette does not require much material or mass. The fibers within the enveloping material or outer tube of the filter are held together by the mechanical interlocking of the fibers with other fibers. The term "fiber" as used herein is used in its usual sense. For example, in *Chemical and Process Technology Encyclopedia*, edited by Douglas M. Considine, published by McGraw Hill Book Company, New York, New York, 1974, at page 476, the term is defined as a sinewy, thread-like object that may be described (1) as long and thin because the length of the fiber may be hundreds or even tens of thousands of times greater than the section dimension of the fiber, (2) as possessing strength to resist elongation and being pulled apart, . . . (5) as capable of interlocking or mechanically bonding with other fibers (like or unlike) to form a matrix of fibers that amplifies the foregoing characteristics.

It is important that the fibers be held together by interlocking or mechanical bonding with other fibers rather than by an adhesive coating on the fibers acting to bond the fibers to each other. It is essential that the fibers be exposed for contact with particulates in the smoke. Unless the fibers are exposed for contact with particulates in the smoke, the positive zeta potential of or on the fibers cannot be utilized to cause coalescence of the colloidally dispersed negative particles in the

smoke to enlarge them and render them more easily filterable.

While good results were obtained with filters made of fibers of alumina, zirconia, alumina-silica, and mixtures thereof, the effectiveness of the filters was improved by further increasing the positive zeta potential of the fibers. This was done by coating the fibers with a secondary source of a positive charge; that is, a positive colloidal metal oxide having more than one positive ion. 5 Preferably, such zeta booster is  $\text{Fe}(\text{OH})_3$ . The advantage of colloidal iron is that it reacts with sulfides such as  $\text{H}_2\text{S}$  and removes it as  $\text{FeS}$  from the mixture of gases. Other booster materials are ammonium or sodium aluminate, sodium zincates, and zinc oxide. The amount of 10 the booster material or materials may be from a trace to saturation of the fibers. It has been found that even a very small amount of the positive zeta potential booster enhances the action of the positively charged fibers.

Where a positive zeta potential booster is used, the 15 fibers selected for the filter are hydrophilic. If the booster is omitted, it is preferred that the fibers be hydrophobic in character.

Although the invention is preferably used as the filter 20 end of a cigarette, a cartridge may be made in accordance with the invention for mounting in a cigarette 25 holder as known in the art.

Although negatively charged particles predominate, tobacco smoke also contains particles which are positively charged and particles which are neutral. The 30 invention contemplates the treatment of the tobacco so that the carcinogenic tars are removed to an even greater extent by treating the tobacco to be associated with the described filter so that upon burning of the tobacco stronger and additional negative charges are 35 imparted to or induced upon the particulate matter of particles in the smoke.

For the foregoing purposes, the divided tobacco for 40 use in a cigarette or the like has mixed therewith particles of a water-insoluble, hydrophobic, moisture-laden, negative charge-inducing or -imparting substance. Materials of this kind presently known may be generally designated as methylated silicas, and are marketed by Cabot Corporation, Boston, Massachusetts 02110 under the trademark "Silanox", and by Degussa, Inc., Kearny, 45 New Jersey 07032 under the trademark "Aerosil". The product made by Cabot Corporation is a trimethylsilyl group on the surface of the base-fumed silicon dioxide particle after reaction with silane. The reaction changes the surface characteristic of the silicon dioxide from hydrophilic to hydrophobic. The formula is  $(\text{CH}_3)_3-\text{Si}-\text{O}-\text{Si}$ . The product made by Degussa is essentially the same except that there are two (2) methyl groups instead of three (3).

In the presence of the hydrophobic, colloidal, negatively charged methylated silica, water is finely dispersed, so that the fine mist-like particles are surrounded by the colloidal silica particles to prevent them from reuniting to form larger particles. A substance is obtained which has the appearance of a dry powder. 55 Such dry powder is best obtained by using approximately 10% of the colloidal silica and 90% water. Objects immersed in this material are not wetted, and this emulsion of water in hydrophobic, colloidal, methylated silica may be described as "dry water".

Divided tobacco to be made into a cigarette is mixed with the described negatively charged hydrophobic, methylated silica-water system, or "dry water", so that the composition is uniformly dispersed throughout the

tobacco. Tobacco thus treated when made into a rod confined by cigarette paper and assembled with a filter made as hereinbefore described furnishes substantially better results than the described filter associated with tobacco which has not been so treated.

The described moisture-laden substance releases moisture upon burning of the tobacco. Tobacco burns at a temperature of approximately 800° C. When drawing upon a cigarette having the tobacco thereof mixed with the described moisture-laden substance, the temperature of the gases or smoke, which is less than the temperature of burning, causes the moisture-laden substance to release the finely dispersed mist-like particles of water, or moisture.

The described filter, and cigarette made with the filter associated with tobacco treated as hereinbefore described act to remove a substantial amount of carcinogenic tars and nicotine; nevertheless, the flavor of the cigarette is not lost because it appears that the flavor-supplying ketones, carbonyls and esters are retained.

Cigarettes made with a filter having alumina fibers in which the fibers were coated with a positive zeta potential booster of ferric hydroxide, and with such filter associated with tobacco treated with "dry water" as hereinbefore described upon smoking tests displayed substantially all the discoloration at the juncture of the filter plug with the tobacco; at the mouth end, the filter was practically clear.

All of the compositions, materials and substances referred to are non-toxic and do not present a health hazard to the smoker.

It is believed that the advantages and improved results afforded by the filter of the invention, and by a cigarette comprising tobacco treated in accordance with the invention associated with the described filter will be apparent from the foregoing description of the preferred embodiment of the invention. Various changes and modifications may be made without de-

parting from the spirit and scope of the invention as sought to be defined in the following claims.

I claim:

1. A filter for tobacco smoke comprising non-toxic, synthetic, inorganic, water-insoluble, anhydrous fibers having a positive zeta potential at the pH of tobacco smoke, the fibers being of a length to enable the interlocking of the fibers, and the fibers being exposed for contact with particulates in the smoke.
2. A filter according to claim 1 wherein the fibers are selected from the group consisting of alumina, zirconia, mixtures of alumina and alumina-silica, and mixtures of zirconia and alumina-silica.
3. A filter according to claim 1 wherein the fibers are hydrophobic.
4. A filter according to claim 1 wherein the fibers are hydrophilic.
5. A filter according to claim 1 wherein the fibers are alumina.
6. A filter according to claim 5 wherein the alumina fibers are hydrophilic and coated with a positive zeta potential enhancing agent.
7. A filter according to claim 6 wherein the positive zeta potential enhancing agent is  $Fe(OH)_3$ .
8. A filter according to claim 5 wherein the alumina fibers have a positive zeta potential at the pH of tobacco smoke of approximately 48 millivolts.
9. A filter according to claim 8 wherein the alumina fibers are hydrophilic and coated with a positive zeta potential enhancing agent.
10. A filter according to claim 1 wherein the fibers are hydrophilic and coated with a positive zeta potential enhancing agent.
11. A filter according to claim 1 wherein the fibers have a positive zeta potential at the pH of tobacco smoke of at least 48 millivolts.

\* \* \* \* \*